

Aug. 9, 1949.

J. J. GREBE

2,478,478

POTENTIAL GRADIENT ANODE FOR GALVANIC PROTECTION

Filed Feb. 3, 1947



Fig. 1



Fig. 3



Fig. 2



Fig. 4



Fig. 5

INVENTOR.  
John J. Grebe

BY

Griswold & Burdick  
ATTORNEYS

## UNITED STATES PATENT OFFICE

2,478,478

POTENTIAL GRADIENT ANODE FOR  
GALVANIC PROTECTIONJohn J. Grebe, Oak Ridge, Tenn., assignor to The  
Dow Chemical Company, a corporation of Dela-  
ware

Application February 3, 1947, Serial No. 725,981

10 Claims. (Cl. 204—197)

1

This invention relates to an improved construction for consumable metal anodes used in the galvanic protection of corrodible metal structures. It also concerns metal protection systems using such anodes.

In the galvanic protection of pipelines and other underground steel structures, consumable electrodes of a metal anodic to the steel are buried in the earth near the structure and are connected to it by electrical conductors. The resulting flow of current maintains the structure cathodic with respect to the soil and greatly minimizes its corrosion. The consumable anodes heretofore used have conventionally consisted of a body of a highly electronegative metal, such as zinc or magnesium, cast about a steel core. Unfortunately, such anodes, while effective, have, in general, exhibited lower overall energy efficiencies than is desirable.

Thus, the consumable anodes, when first installed, must develop a comparatively high current in order to protect the structure. Then gradually, as the structure becomes polarized, much less current is needed. The conventional anodes, however, because of their construction, develop a nearly constant potential, and hence roughly constant current, throughout most of their life. They thus tend, over a long period, to supply considerably more current than is actually required by the structure. This excess current, of course, consumes a part of the active metal of the anodes. If attempt is made to limit the current after the initial stages by inserting resistances in the circuit, the anodes are forced to operate at low current densities, under which conditions self-corrosion or pitting of the active metal is often severe. In addition, once the consumption of the active metal proceeds to a point where the steel core is partly exposed, a strong electrolytic couple is set up within the anode which further accelerates self-corrosion of the remaining active metal. All these factors are reflected in varying degree in the overall energy efficiencies observed with conventional anodes.

In view of these considerations, it is an object of the present invention to provide a consumable anode for use in galvanic protection which develops a single-electrode potential that decreases as the anode is consumed. Another object is to provide an efficient anode which is consumed uniformly, with but little pitting or self-corrosion even at low current densities. An additional object is to provide an anode in which the core tends to remain unexposed until the active metal is virtually all consumed.

These objects are realized according to the invention by a consumable anode, the body of which is formed of an alloy of an anodically active metal in which the proportion of such metal

2

decreases from the outside of the body to the core. With such an electrode, the inner portions are less anodic than the surface. Consequently, as the electrode is consumed, the potential developed, and the current output in a given installation, decline gradually. Further, with the outer portions of the electrode anodic to the underlying metal, the electrode is of necessity consumed from the outside inwardly in a uniform and efficient manner; pitting is very greatly minimized, and exposure of the core seldom occurs.

The invention may be illustrated with reference to the accompanying drawing, in which

Fig. 1 is a transverse section through a consumable anode according to the invention, with zone-wise variation in alloy composition;

Fig. 2 is a longitudinal central section through the anode of Fig. 1;

Fig. 3 is a transverse section through an alternative form of anode, with continuous variation in alloy composition;

Fig. 4 is a longitudinal central section through the anode of Fig. 3; and

Fig. 5 is a diagrammatic vertical section showing the manner of using a consumable anode in the galvanic protection of a buried pipeline.

Consumable anodes according to the invention consist of a body of alloy of an anodically active metal with a less active metal, which body surrounds and is firmly bonded to an electrically conductive core of a material different from and cathodic to that of the body. The proportion of active metal in the alloy decreases, either zone-wise or in continuous progression, from the outside of the body to the core.

The active metal forming the alloy may be any of the more highly electronegative metals commonly used in consumable anodes for galvanic protection work, especially magnesium or zinc. The less active metal component of the alloy may, so far as known, be any metal cathodic to and alloyable with the active metal, e.g. aluminum or zinc in the case of magnesium as the active metal. The preferred anodes are formed of alloys of the magnesium-aluminum system.

The core of the anode may, in conventional manner, be of any electrically conductive and preferably also mechanically strong material different from and cathodic to that of the body.

In the case of magnesium alloy anodes, a non-magnesian metal core is preferred, mild steel rod or cable being convenient.

A preferred form of the consumable anodes of the invention, with zone-wise variation in alloy composition, comprises an elongated metal core surrounded by and bonded to an elongated body of magnesium-aluminum alloy in the form of two or more annular zones of differing magnesium content all concentric with the core, the cross-sectional area of each zone being a substantial

fraction of that of the entire body and the proportion of magnesium in the metal in any zone being greater than that in the zone nearer the core.

In a particularly advantageous construction, using two zones, a steel rod core is surrounded by an annular body of an alloy containing from about 1 to about 92 percent by weight of magnesium, balance substantially aluminum, this latter being in turn surrounded by another annular body of a metal containing more than 95 percent by weight of magnesium, the cross-sectional area of each body being large in comparison to that of the core. In this anode, the alloy of the outside zone, being essentially magnesium, provides a high electrolytic potential and is virtually non-polarizing in use. The central alloy zone, with 1 to 92 percent magnesium, is of readily polarizable material. As the anode is consumed and this zone is exposed, the alloy, because of this polarization, as well as the fact that it is cathodic to the outer layer, remains virtually unattacked until the more magnesium-rich layer is entirely gone. At that time, the central zone then begins to deliver current at a lower potential and a reduced output.

It is highly desirable that the alloy composition of the inner zone be controlled within the limits of 1 to 92 percent magnesium. If the lower limit is passed, the alloy approaches pure aluminum in behavior and is subject to substantial cathodic corrosion and pitting by the alkaline medium produced as the outer magnesium zone is consumed. If the upper limit is exceeded, the alloy behaves much like magnesium, does not polarize readily, and is not sufficiently cathodic with respect to the outer metal. Optimum construction calls for an anode having an inner zone of an aluminum-base alloy containing from 1 to 12 percent by weight of magnesium as the major alloying element and an outer zone of a metal containing more than 95 percent of magnesium. An anode of this character is illustrated in Figs. 1 and 2, in which a mild steel core is bonded to an inner zone of a commercial aluminum-base alloy containing about 4 percent magnesium, balance substantially aluminum, the outside zone being commercially pure magnesium.

Zone-wise anodes as in Figs. 1 and 2 may be produced in any of several ways. In one method, a clean steel core, preferably galvanized to assure good bonding, is centered axially in a cylindrical mold and the alloy of the inner zone is cast around it. The resulting body, after cooling, is centered in a larger cylindrical mold and the metal of the outer zone cast around it. Diffusion and even intermelting of the metal of the two zones occur at the interface, providing solid bonding. Another method of making the anodes consists in separately casting the inner zone with its core and the annular outer zone and then shrinking the latter on the former. Alternatively, the anodes may be produced by the techniques of powder metallurgy, or by making an appropriate composite tubular extrusion by the process of U. S. 2,023,498, fitting the steel core in place, and forging the whole lightly to insure good bonding throughout. Each of these methods is equally applicable to making anodes consisting of three or more annular zones of differing magnesium content.

An alternative form of anode according to the invention, with continuous rather than of zone-wise change in alloy composition, is illustrated schematically in Figs. 3 and 4. In this anode,

the steel core is bonded to a body of a magnesium-aluminum alloy in which the proportion of magnesium decreases in fairly uniform progression from the outside of the body to the core. In such anodes, the alloy nearest the core is preferably rich in aluminum while the outside metal may be nearly pure magnesium. Such anodes are best made by first producing a zone-wise anode, as already described, and then subjecting it to a diffusional heat-treatment at a temperature of 400° to 800° F. for a period of 24 hours or more. At these temperatures, the aluminum and magnesium of the various zones interdiffuse slowly, producing a body in which the magnesium content decreases progressively from the outside inwardly.

The consumable anodes of the invention are used in galvanic protection systems in conventional manner in place of the anodes heretofore used, and exhibit exceptional advantages, as already explained. In a typical installation, illustrated in Fig. 5, an anode of the preferred type shown in Figs. 1 and 2 is used in the galvanic protection of a steel pipeline buried in the earth. As shown, the anode is buried in a suitably-sized hole in the earth a short distance from the pipeline and is surrounded by a backfill, such as a bentonite-gypsum mixture, which serves to control the anode environment. An insulated wire electrically connects the core of the anode to the pipeline.

While the anodes are particularly useful in the protection of underground ferrous metal structures, they may be employed generally in the galvanic protection of ferrous metals immersed in natural aqueous electrolytes, including ground water, fresh water, and seawater. It is necessary only that one or more anodes be immersed in the same body of electrolyte as the structure and be connected electrically to the latter. Typical uses are the protection of ships' bottoms and the prevention of corrosion of domestic hot water heaters. The criteria for choosing the size and number of anodes for a given installation are well known in the art.

It is understood that the foregoing description is illustrative rather than limitative, and that the invention is co-extensive in scope with the following claims.

50. What is claimed is:

1. A consumable anode for use in galvanic protection of metallic structures comprising a body of alloy of an anodically active metal with a less active metal, both such metals being anodic with respect to the metal of the structure to be protected, such body having therein an electrically conductive core of a material different from and cathodic to that of the body, the proportion of more active metal in the alloy forming the body decreasing from the outside of the body to the core.

2. A consumable anode for use in galvanic protection of ferrous metal structures comprising a body of alloy of magnesium with a less anodic metal which is anodic to the ferrous metal of the structure to be protected, such body having therein a core of non-magnesian metal cathodic to that of the body, the proportion of magnesium in the alloy forming the body decreasing from the outside of the body to the core.

3. An anode according to claim 2 wherein the body is formed of a binary magnesium-aluminum alloy.

4. An anode according to claim 2 wherein the core is made of steel.

5. A consumable anode for use in galvanic protection of metallic structures comprising a steel core surrounded by and bonded to a body of magnesium-aluminum alloy, the proportion of magnesium in the alloy forming the body decreasing in continuous progression from the outside of the body to the core.

6. A consumable anode for use in galvanic protection of ferrous metal structures comprising an elongated body of magnesium-aluminum alloy surrounding and bonded to an elongated core of non-magnesic metal cathodic to that of the body, the body being the form of a plurality of annular zones of differing magnesium content concentric with the core, the cross-sectional area of each zone being a substantial fraction of that of the entire body and the proportion of magnesium in the metal in any zone being greater than that in zones nearer the core.

7. An anode according to claim 6 wherein the core is made of steel.

8. A consumable anode for use in galvanic protection of metallic structures comprising an elongated steel core surrounded by and bonded to an annular alloy containing from about 1 to about 92 percent by weight of magnesium, balance substantially aluminum, such body being surrounded by and bonded to an annular body of a metal containing more than 95 percent by weight of magnesium, the cross-sectional area

5

15

25

30

of each body being large in comparison to that of the core.

9. A consumable anode for use in galvanic protection of metallic structures comprising an elongated steel core surrounded by and bonded to an annular body of an aluminum-base alloy containing from at least 1 percent to 12 percent by weight of magnesium as the major alloying element, such body being surrounded by and bonded to an annular body of a metal containing more than 95 percent magnesium, the cross-sectional area of each body being large in comparison to that of the core.

10. In combination with a ferrous metal structure immersed in a natural aqueous electrolyte, galvanic protection means comprising an anode as defined in claim 1 immersed in the electrolyte near the structure and electrically connected to the same.

JOHN J. GREBE.

#### REFERENCES CITED

The following references are of record in the file of this patent:

#### UNITED STATES PATENTS

| Number    | Name         | Date          |
|-----------|--------------|---------------|
| 2,011,613 | Brown et al. | Aug. 20, 1935 |
| 2,204,823 | Rhodes       | June 18, 1940 |